

Patented Sept. 18, 1934

1,973,788

# UNITED STATES PATENT OFFICE

1,973,788

## METHOD OF OBTAINING PHOTOGRAPHIC CONTRASTS BY MEANS OF DIAZONIUM COMPOUNDS

Roelef Jan Hendrik Alink and Jan Hendrik de Boer, Eindhoven, Netherlands, assignors to N. V. Philips Gloeilampenfabrieken, Eindhoven, Netherlands

No Drawing. Application November 10, 1932, Serial No. 642,124. In the Netherlands November 10, 1931

7 Claims. (Cl. 95—7)

The present invention relates to improvements in the method of obtaining photographic contrasts by means of diazonium compounds described in the co-pending application Ser. No. 612,364 filed May 19, 1932 of de Boer, Dippel and Alink.

In the above referred to application there is described a novel method of obtaining photographic contrasts by means of diazonium compounds which instead of being based on the production of azo dyes by coupling of a diazonium compound with an azo component—utilized in previously known methods of obtaining diazo-types—utilizes the oxidizing properties of certain diazonium compounds. Thereby colored oxidation products are formed from the light-decomposed products of the diazonium compounds.

According to the process of the above referred to application, a carrier is provided with a light sensitive substance which consists of one or more diazonium compounds of which compounds at least one, upon exposure to actinic light in the presence of water, forms a phenol so substituted in the benzene nucleus, that the phenol can be oxidized either by the non-decomposed portion of that particular diazonium compound or by some other diazonium compound provided on the carrier. A colored compound is thus formed without the addition of an azo component, whereby the diazonium compound oxidizes the phenol produced during the exposure much more rapidly than it would couple therewith to form an azo dye.

In this process, as stated in the above application, such diazonium compounds have been found especially suitable, which yield after their exposure polyphenols which are in no way capable of coupling with diazonium compounds. For example, a suitable compound for printing paper is parahydroxy - benzene - diazoniumchloride, upon exposure of which hydroquinone, nitrogen and hydrochloric acid are formed.

Another suitable diazonium compound is, for instance, 1-hydroxy-2-diazo-4-benzenesulphonic acid.

The process of making heliographic prints by means of a carrier provided with a light sensitive diazonium compound described in the above application consists in locally exposing such carrier to a light having a strongly actinic effect on the light sensitive substance, after which the whole carrier is subjected to a second exposure, this time to a light which is only slightly actinic with regard to the light sensitive substance of the carrier, so that part of the diazonium compound

is converted into a phenol and this phenol is caused to be oxidized by the non-converted portions of the diazonium compound to form a colored oxidation product. The oxidization may be accelerated by moderate heating to about 80° C. 60 and the formation of contrasts can be greatly promoted by the addition of copper salts, such as copper nitrate. Excellent contrasts are obtained on a positive print made from a positive, for instance from a drawing, if the paper serving 65 as carrier is soaked in a 0.25% alcoholic solution of -1-hydroxy-2-diazo-4-benzene-sulphonic acid, to which 0.55% of copper nitrate is added. After the paper is dried, the print is made by exposing the so treated carrier under the drawing to the 70 light of a suitable highly actinic light source, for instance a carbon arc lamp, for about 20 seconds, and after such exposure the paper is exposed to regular light and preferably heated for a certain period at about 80° C. Thereby a positive 75 print having a dark steel gray tone is obtained from the drawing.

Thus, as more fully described in the above application, in this method which is based on the oxidation of the product produced by exposure 80 from the diazonium compound by a still unconverted diazonium compound, no substance needs to be added after the exposure, nor needs the print to be subjected to further treatments.

The advantages of this novel method are simplicity, low cost and at the same time excellent prints are obtained.

The present invention relates to an improvement in the method of the above application.

As light sensitive carriers, for instance, printing paper, are generally stored for a considerable time prior to their use they are generally kept in closed containers to prevent access of light. It has been found however that a light sensitive carrier, for instance, printing paper made according to the prior invention, when subjected to prolonged storage in such containers decreased in light-sensitivity and after several months the paper loses practically all of its light-sensitivity.

Experiments have shown that this loss in light-sensitivity is not due to the access of light or oxygen but to moisture either present in the paper or gradually absorbed from the air even when the container was kept closed or when it was opened (without access of light) for short periods to remove some of the paper. Even a small amount of moisture had a considerable deteriorating effect, which is due to some chemical reaction probably in the form of the diazonium 110

group being replaced by a hydroxyl group. It was found that when such paper was exposed to a very damp medium, the annihilation of the diazonium group took place so rapidly that the diazonium compound which has been converted by water could no more be oxidized by the unconverted diazonium compound. Paper which had lost all its light-sensitiveness in this way showed a practically white color over its entire surface.

10 Further experiments showed that if only a small amount of water vapor or water was allowed to act on such light sensitive paper, its light sensitiveness could be longer maintained. However, even in this case the light-sensitiveness is eventually entirely lost, but in this case the paper, after losing its light sensitiveness, showed a dark color. This may be due to the oxidation of the gradually produced oxidizable phenol by diazonium compound not yet decomposed by the water and of which a plentiful supply is still present as the reaction takes place gradually.

15 It was found, furthermore, that such sensitized paper will maintain its light sensitiveness almost indefinitely if it is highly dried and stored in a highly dry atmosphere, this being even the case when oxygen is present. On the other hand, an exhausted and air-tightly sealed container would not protect the light sensitiveness of the paper if water vapour is present in the container.

20 The present invention, therefore, relates to a method of drying a light-sensitive material, for instance, heliographic printing paper, made according to the invention of the prior application, to remove from it the moisture to such extent that chemical reactions conducive to the deterioration of the light sensitive properties of the material be prevented and to maintain said material in such a dry state during its storage.

25 While it is known practice to dry certain types of papers, for instance, light sensitive papers used for printing, and keep them reasonably dry in storage or dry them before use, a small amount of moisture present in such papers does not deleteriously influence their properties.

30 However, in the present instance, the light sensitive material, made according to the invention of the prior application, permanently deteriorates in the presence of even a small amount of moisture and to maintain its initial and maximum light sensitivity it has to be dried and kept dry to a greater extent than is the practice in drying paper, and to a greater extent than it is possible with the generally used drying methods.

35 According to the invention, the moisture content of the light sensitive material is reduced to less than 1%, and the paper maintained during its storage in such dry condition whereby the decomposition of the diazonium compound is altogether prevented and the light sensitiveness of the material made according to the invention of the prior application can be maintained to its full extent.

40 The above definition of the moisture content will be fully understood from the following:

45 If a so-called air-dried paper is subjected to the well-known drying process of heating it at a temperature between 105 to 110° C. for 24 hours, it shows a decrease of between 5 to 6% in weight, such decrease not exceeding 6.5%.

50 On the other hand, if such air-dried paper is placed in a container comprising fresh phosphorus-pentoxide and is maintained in the container for 24 hours at a temperature of about 75 25° C., it shows a decrease in weight of about 8%.

A paper dried by the second method can be regarded as bone dry, and the sensitized paper to fulfill the above stated condition should be deprived from moisture to such extent as to lose about 7% of its weight compared to its air-dry condition.

55 According to one method of our invention a suitable paper, after being sensitized by means of an alcoholic solution of a diazonium compound of the nature above described, is dried under vacuum until its moisture content has been reduced to the above extent.

60 Another method provides for the drying of such a sensitized paper in an enclosure which has an atmosphere maintained perfectly dry by a powerful drying agent, for instance, by phosphorus-pentoxide.

65 In a still further method of drying, the sensitized paper is placed in a container and flushed with a gas, for instance, nitrogen or air, from which all moisture has been extracted either by means of a powerful drying medium, for instance, phosphorus-pentoxide, or by freezing the moisture out at a very low temperature. For instance, from air moisture can be completely frozen out at about -180° C.

70 Of if desired, combinations of the above drying processes may be used.

75 To maintain the paper so dried during its storage in its highly dry condition, we provide for it containers, for instance glass receptacles which are sealed by a moisture-proof compound, for instance, a suitable sealing wax, and which container does not comprise moisture at all or the moisture content of which is so low that the paper can absorb no such quantities of moisture which would increase its moisture content above 1%.

80 Again, the dried light sensitive material may be stored in hermetically-sealed metal boxes or containers consisting of thin metal plates, the edges of which are welded or soldered together, and which have been freed from moisture.

85 It should be pointed out that the generally used wrapping means, for instance, cardboard containers or paraffin impregnated paper wrappers, which are entirely suitable containers for other light sensitive materials, are deficient as containers or wrappers for light sensitive material according to the prior application, and even if such light sensitive material has been sharply dried by one of the previously described methods, sufficient moisture will gain access to it and gradually destroy its light sensitive properties.

90 It should be also understood that if the light sensitive material when placed in the container is provided with a protective wrapping of ordinary paper or similar material, such wrapping paper has also to be dried to a similar extent as the light sensitive material.

95 While prolonged drying under a high temperature might expel sufficient moisture from the light sensitive material to reduce its moisture content within the above stated limit, drying by heat is as a rule objectionable as at elevated temperatures a partial decomposition and oxidation of the diazonium compound takes place.

100 By the high degree drying and keeping the material in such highly dried condition, deterioration of the light sensitive material is wholly prevented, and the contrasts obtained in printing are very sharp whereby the copied out portions of the print are and remain white. At the same time the light sensitiveness of the paper is much greater when in such highly dry state than in the case when it has a moisture content exceeding 1% and thus a much shorter exposure can

be used with highly dried paper than with a paper having such higher moisture content, and this holds irrespective of the time of storage of such paper.

5 While we have described our invention with reference to certain examples, it should be well understood that we do not wish to be limited to such, but desire the appended claims to be construed as broadly as permissible in view of the prior art.

What we claim is:

1. The method of producing a light-sensitive material comprising a diazonium compound which upon exposure to actinic light in the presence of water forms a phenol which is oxidized by the unconverted portions of a diazonium compound and forms a colored compound without the addition of an azo-component, comprising the steps of providing a carrier with said diazonium compound and removing from said material the moisture so that it forms less than 1% of the weight of the material.

2. The method of producing a light-sensitive material comprising a diazonium compound which upon exposure to actinic light in the presence of water forms a phenol which is oxidized by the unconverted portions of a diazonium compound and forms a colored compound without the addition of an azo-component, comprising the steps of providing a carrier with said diazonium compound and removing from said material the moisture so that it forms less than 1% of the weight of the material and enclosing said material in an air tightly sealed container having a substantially moisture-free atmosphere.

3. The method of producing a light-sensitive material comprising a diazonium compound which upon exposure to actinic light in the presence of water forms a phenol which is oxidized by the unconverted portions of a diazonium compound and forms a colored compound without the addition of an azo-component, comprising the steps of providing a carrier with said diazonium compound and placing said material in a closed container, evacuating said container to remove from said material the moisture so that it forms less than 1% of the weight of the material.

4. The method of producing a light-sensitive material comprising a diazonium compound which upon exposure to actinic light in the presence

ence of water forms a phenol which is oxidized by the unconverted portions of a diazonium compound and forms a colored compound without the addition of an azo-component, comprising the steps of providing a carrier with said diazonium compound and subjecting said material to a drying operation by flushing it with a gas free from moisture to remove from said material the moisture so that it forms less than 1% of the weight of the material.

5. The method of producing a light-sensitive material comprising a diazonium compound which upon exposure to actinic light in the presence of water forms a phenol which is oxidized by the unconverted portions of a diazonium compound and forms a colored compound without the addition of an azo-component, comprising the steps of providing a carrier with said diazonium compound and subjecting said material to a drying operation by flushing it with a gas from which the moisture has been removed by freezing it out at low temperature to remove from said material the moisture so that it forms less than 1% of the weight of the material.

6. The method of producing a light-sensitive material comprising a diazonium compound which upon exposure to actinic light in the presence of water forms a phenol which is oxidized by the unconverted portions of a diazonium compound and forms a colored compound without the addition of an azo-component, comprising the steps of providing a carrier with said diazonium compound and subjecting said material to a drying operation by flushing it with a gas from which the moisture has been removed by freezing it out at about -180° C. to remove from said material the moisture so that it forms less than 1% of the weight of the material.

7. A light-sensitive material comprising a carrier such as paper provided with a light-sensitive layer, in which the light sensitive substance comprises a diazonium compound which upon exposure to actinic light in the presence of water forms primarily a phenol so substituted in the benzene nucleus that this phenol can be oxidized by an unconverted diazonium compound to form a colored compound without the addition of an azo-component, said material having a moisture content less than 1%.

ROELOF JAN HENDRIK ALINK. 125  
JAN HENDRIK DE BOER.